

# United States Patent

[19]

Ohtomo et al.

[11]

3,996,327

[45]

Dec. 7, 1976

[54] **PROCESS FOR SPINNING COMPOSITE FIBER OF PHENOLIC RESIN**

[75] Inventors: **Koichiro Ohtomo**, Takatsuki; **Thuyoshi Nakamori**, Osaka, both of Japan

[73] Assignee: **Nippon Kynol Inc.**, Osaka, Japan

[22] Filed: **Oct. 14, 1975**

[21] Appl. No.: **621,846**

## Related U.S. Application Data

[63] Continuation of Ser. No. 424,696, Dec. 14, 1973, abandoned.

## Foreign Application Priority Data

Dec. 20, 1972 Japan ..... 47-127905  
Oct. 15, 1973 Japan ..... 48-115511

[52] U.S. Cl. ..... **264/168; 264/171; 264/236; 428/369; 428/374**

[51] Int. Cl. <sup>2</sup> ..... **B29F 3/10**

[58] Field of Search ..... 428/369, 374; 264/168, 264/171, 236

[56]

## References Cited

### UNITED STATES PATENTS

|           |         |                      |         |
|-----------|---------|----------------------|---------|
| 3,639,953 | 2/1972  | Kimura et al. ....   | 264/29  |
| 3,651,199 | 3/1972  | Blume et al. ....    | 264/347 |
| 3,808,289 | 4/1974  | Okuhashi et al. .... | 260/841 |
| 3,928,526 | 12/1975 | Koyama ....          | 264/347 |
| 3,931,386 | 1/1976  | Kimura et al. ....   | 264/347 |

Primary Examiner—Jay H. Woo  
Attorney, Agent, or Firm—Sherman & Shalloway

[57]

## ABSTRACT

A method of producing a self-crimping composite fiber of phenolic resin having heat-resistant and flameproof properties which comprises compositely spinning a thermoplastic phenolic resin and a modified phenolic resin consisting of a thermoplastic resin and another thermoplastic resin, such that the two components are united in either an eccentric or side-by-side arrangement, and thereafter curing the resulting thermoplastic composite fiber.

18 Claims, No Drawings

## PROCESS FOR SPINNING COMPOSITE FIBER OF PHENOLIC RESIN

This is a continuation of application Ser. No. 424,696, filed Dec. 14, 1973, now abandoned.

This invention relates to a method of producing a self-crimping phenolic composite fiber excelling in heat resistance and is flameproof.

The fiber obtained by fiberizing, by means of the melt-spinning process, either a phenolic resin or a heat-meltable material consisting predominantly of such resin and thereafter carrying out the crosslinking reaction by utilizing subjecting its phenol ring to the three-dimensionalized cure of the fiber has been known in the past as being a flameproof fiber.

For instance, the cured phenolic resin fiber obtained by melt-spinning the novolak resin obtained by the condensation of phenol and formaldehyde and thereafter carrying out the crosslinking of the resulting fiber with a combined solution of hydrochloric acid and formalin has the properties of being heat infusible and solvent insoluble, as well as being flameproof. Thus, this fiber can be recommended as being a fibrous material suitable for use in places where fire hazards exist, e.g., for use in the interior decoration field or as flameproof clothings.

However, since this phenolic fiber has been cross-linked to a high degree, it is usually brittle. Hence, in spinning the staples of this fiber, great difficulty is experienced not only when it is spun alone but also when it is mixed spun with other fibers. In addition, not only does the resulting yarn have a small elongation, but also the properties of the final product are not satisfactory. On the other hand, when this fiber is used as a filament yarn, the resulting knit or woven fabric usually has a cold feel and, again, the fabric does not have elasticity. For this reason, there are studies underway to find a method of imparting mechanical crimps to this phenolic fiber but because of the foregoing brittleness, considerable difficulty is involved.

The melt-spinning of the phenolic resins is difficult, as a rule. For solving this problem, the method of spinning the phenolic resins after mixing them with other heat-meltable resins is known. However, for achieving good spinnability in this case, a considerably large amount of the other heat-meltable resin must be admixed. As a consequence, there is the drawback that a great drop is brought about in the flame resistance, the characteristic feature of the phenolic resins.

As a consequence of our extensive research with a view to solving the various foregoing deficiencies of the conventional techniques, we arrived at the present invention.

An object of the present invention is to provide a self-crimping phenolic fiber which not only has good spinnability but also excels in elongation and recovery. Another object is to improve the spinnability of the phenolic resins without impairing the heat-resistant and flameproof properties of these resins.

Accordingly, the present invention is directed to a method of producing a self-crimping phenolic composite fiber having heat-resistant and flameproof properties, which comprises melt-spinning (a) a modified phenolic resin obtained by melt blending a heat-meltable phenolic resin with 0.5 -30 % by weight, based on the total weight of the mixture, of a heat-meltable fiber-forming resin other than phenolic resins, and (b) a

heat-meltable phenolic resin such that the components (a) and (b) are united in an eccentric or side-by-side relationship, and thereafter submitting the resulting heat-meltable composite fiber to a treatment which cures the phenolic resin component contained therein.

Hitherto, a method of developing crimps by treatment of a composite filament composed of two components of differing shrinkability united in either an eccentric or side-by-side relationship, i.e., one in which the components are arranged and united continuously in the lengthwise direction of the filaments in an eccentric or side-by-side relationship over the cross section of the filament with hot water, for example, is being practiced, but in this method the stability of the crimps is low. On the other hand, the invention method comprises subjecting the heat-meltable fiber obtained by the composite spinning to a curing treatment to three-dimensionalize the phenolic resin component contained in the fiber thereby to impart crimpability to the fiber. Hence, the invention method is an entirely new method. It is possible according to the present invention to control the degree of development of crimpability and the time of appearance of the crimps in accordance with the aforesaid curing conditions and the degree of the cure.

The phenolic resins preferably used in the method of this invention are those usually of a molecular weight ranging from 500 to 3000 obtained by the condensation reaction by heating phenol or at least one of such phenols as cresol, p-tert.butyl phenol or chlorophenol, and the so-called aldehydes such as formaldehyde, paraformaldehyde, hexamethylenetetramine and furfural, in the presence of an inorganic or organic acid catalyst such as hydrochloric acid, sulfuric acid, phosphoric acid, p-toluenesulfonic acid and phenolsulfonic acid. Hence, these resins usually consist predominantly of novolak, but there is imposed no restriction at all as to their molecular weight, degree of polymerization or structure as long as they are heat meltable. Resol may also be contained in part in the phenolic resin.

As the various other heat-meltable resins other than the phenolic resins that can be used in the invention method, included are the fiber-forming polymers such, for example, as the polyamides, polyesters, polyurethanes and polyolefins. As the polyamide polymers, mention can be made of such, for example, as nylon 6, nylon 7, nylon 11 and nylon 12, as well as the polyamides obtained by the polymerization of a dicarboxylic acid having an aliphatic, aromatic or alicyclic nucleus, such as adipic acid, sebacic acid, terephthalic acid and isophthalic acid or the hydrogenation products thereof, with a diamine such as ethylenediamine, hexamethylenediamine, nonamethylenediamine, undecamethylenediamine, xylylenediamine or piperazine. The polyesters include polyethylene terephthalate as well as polyoxybenzoate, or the copolymers having these as one of their components. As the polyolefins, mention can be made of polyethylene, polypropylene and polystyrene. Or, when nonflammability is especially desired in the composite fiber product, coal tar or asphalt pitches and resol containing upwards of 15 % of methanol can also be used.

When considered from the compatibility with the phenolic resins, the polyamide are especially preferred among the foregoing resins, and particularly to be preferred is a polyamide which not only has a melting point not exceeding 250° C. but is acid resistant as well. The reason is that in the case of polyamide having a

melting point exceeding 250°C., elevated temperatures are required for its mixing with the phenolic resins, with the consequence that the spinnability of the phenolic resins tends to become poor. On the other hand, in the case of a polyamide having poor resistance to acids, hydrolysis of the polyamide is set up at the time of the hereinafter-described curing treatment that is carried out in accordance with the present invention, with the consequence that the yarn quality of the finally obtained cured phenolic composite fiber is unsatisfactory. Hence, usually used is a polyamide which, when tested by introducing a fibrous polyamide into a 5 weight % aqueous hydrochloric acid solution and treated for 1 hour at 50°C., has a weight loss of less than 25%, preferably less than 10%, and most preferably less than 5%. Further, the foregoing heat-meltable resins can also be used as mixtures of two or more classes thereof.

In preparing the modified phenolic resin component (a) by melt blending the foregoing heat-meltable resins with the phenolic resins, the two components may be mixed in advance in a melt-blending extruder or the two components may be directly fed in, say, chip form to the extruding spinning machine at the time of spinning of the composite fibers.

The heat-meltable resin is added to the phenolic resin in an amount, based on the total amount of the mixture, of 0.5–30% by weight, preferably 1–10% by weight, and most preferably 2–7% by weight. When the heat-meltable resin is added in an amount of less than 0.5% by weight, adequate crimping cannot be obtained, whereas when this amount exceeds 30% by weight, the crimping and spinning properties are satisfactory but, on the other hand, the nonflammability of the resulting products is inadequate, and hence this is undesirable from the standpoint of imparting heat resistance and flameproofness to the product.

The so obtained modified phenolic resin (a) containing a suitable amount of a heat-meltable resin is then spun along with a phenolic resin (b) simultaneously from the same hole of a known composite spinneret, following which the spun filament is wound up in customary manner while being cooled. As regards the form in which the components are united, either the side-by-side or the eccentric core-sheath form will do. Again, the weight ratio of (a) to (b) may be chosen optionally. For instance, this ratio may be 10/90–90/10, and preferably 20/80–80/20, especially preferred being a ratio ranging from 40/60–60/40.

However, when it is intended in this case to improve the spinnability of the fiber as much as possible by using the heat-meltable resins other than the phenolic resin in an amount in excess of 10 parts by weight and further to use the resulting composite fiber in the form of a filament yarn, preferred instead of the side-by-side form is the eccentric core-sheath form which consists of a core of the modified phenolic resin (a) and a sheath of the phenolic resin (b). In this case a much more improved nonflammability can be achieved. Again in the case of the side-by-side arrangement, measures must be taken to ensure that the nonflammability is not impaired by suitably varying the ratio of the components (a) and (b) that are united.

The heat-meltable composite fiber obtained by the melt-spinning operation is then submitted to a curing treatment thereby three-dimensionalizing the phenolic resin contained in the fiber to thus develop the crimps. Preferred modes of carrying out the curing treatment will be described below.

The heat-meltable composite fiber is immersed and held, for example, for 0–2 hours at room temperature in a combined aqueous solution containing 0.1–25% by weight of a catalyst selected from the inorganic acids such as hydrochloric acid and sulfuric acid, or an organic acid such as formic acid, benzenesulfonic acid, toluenesulfonic acid and phenolsulfonic acid and 0.5–35% by weight of such aldehydes as are typified by formaldehyde, after which the temperature of the solution is raised up to 50°–105°C. thereby curing the phenolic resin contained in the sheath layer of the fiber. The state of the crimps (number of crimps and size) can be freely adjusted by varying the rate of temperature rise, the maximum temperature used and the concentration of the curing bath. Generally speaking, the degree of crimping obtained increases as the rate of temperature rise, maximum temperature used and concentration of the curing bath become higher. Next, after raising the temperature, the heat treatment is continued for a further 0.1–40 hours at 50°–105°C. thereby effecting a still greater stabilization of the crimps, as well as to cause the fiber to become insoluble and infusible and to render it nonflammable. While it is preferred to usually use the curing agents such as indicated hereinbefore in the curing treatment, it is also possible to incorporate in advance in the heat-meltable resin a reagent which forms an aldehyde on thermal decomposition, such, for example, as tetraoxane, and cure the phenolic resin by the thermal decomposition of this reagent.

On the other hand, as another procedure it is possible to carry the cure to the interior of the fiber by the following procedure. In the first stage of the curing treatment described above the time at which the temperature is held at 50°–105°C. after raising the temperature is held to within 0–2 hours to effect partial cure of the sheath layer. Then as the second stage of the curing treatment the fiber is immersed at room temperature in a combined aqueous solution containing 0.2–15% by weight of a basic catalyst such as ammonia or an amine and 1–40% by weight of an aldehyde, followed by raising the temperature to 70°–90°C., at which temperature the reaction is continued for a further 0.5–10 hours. By this two-stage curing treatment a composite fiber in which the degree of crimp and stability of the crimps are enhanced somewhat can be obtained.

In carrying out the foregoing second stage curing treatment, it is possible to incorporate either the urea bond or the thiourea bond in the crosslinked phenolic resin molecules by using as the curing treatment liquid a combined solution of either an acid catalyst or a basic catalyst and an aldehyde in which has been incorporated a small amount of either urea, thiourea or a methanol derivative thereof, whereby it becomes possible to provide a composite fiber which is thermally infusible, solvent insoluble and nonflammable, and excelling especially in heat resistance.

Thus, in accordance with the present invention, as a consequence of having submitted the composite heat-meltable resin fiber to a curing treatment, a self-crimping nonflammable phenolic composite fiber can be obtained. For forming in this case a composite fiber having firmly set crimps and excelling in elongation and recovery, the crosslinking of the phenolic resin component by means of the curing treatment must not be excessive. The degree of crosslinking suitable in the case of the invention method is 5–45 mol %, and pref-

erably 10–35 mol %. By the expression "degree of crosslinking," as here used, is meant the degree of tri-substitution of the phenol nucleus contained in the resulting composite fiber, and this can be readily calculated by using the infrared spectrum. When the degree of crosslinking is less than 5 mol %, the crimps obtained are weak and the elongation recovery is poor. On the other hand, when 45 mol % is exceeded, the degree of crosslinking being too high, this also is undesirable, since the yarn quality suffers. A degree of crosslinking coming within the foregoing range can be realized by employment of the hereinbefore-indicated curing conditions.

Now, in practicing the hereinbefore-described curing treatment on a large commercial scale, it frequently happens that agglutination between the individual filaments takes place in the curing bath. This must be especially guarded against. Especially in the case where the curing treatment is carried out by the batch method wherein the packing density of the filaments is high, as a consequence of the shrinkage of the filaments that takes place in concomitance with the formation of crimps, the filaments become adhered to each other to cause at the same time a nonuniform curing of the filaments. Hence, this results in hindering the smooth operation of the cure, and this makes it difficult to obtain products of good quality. For avoiding this difficulty, either the packing density of the filaments must be reduced or the continuous method wherein the filaments are fed in small amounts continuously must be employed. However, as a result of extensive research, a much more improved method has been found. This new method consists fundamentally of avoiding the agglutination of the filaments from taking place by inhibiting as much as possible the development of the crimps in the curing bath and thereafter treating the resulting cured composite filaments with a swelling agent, thereby developing the desired crimps. In other words, the crimps are kept as much as possible in their latent state in the filaments during the curing process and are then developed and made manifest in the following swelling process. This method provides good quality products having much more uniform crimps.

The inhibition of crimp development in the curing bath can be achieved by an adjustment of the curing conditions to be employed, as by the use of a curing bath of suitable composition and employment of a relatively mild rate of temperature rise and maximum temperature. These curing conditions and a preferred mode of carrying out the swelling treatment will be more fully described below. In the following description the acidic and basic substances used as catalyst in the curing bath, as well as the aldehydes used therein as the curing agent are the same as those hereinbefore mentioned, and the percentages thereof are on a weight basis.

The first stage curing treatment is carried out by immersing the heat-meltable composite fiber at room temperature in a curing bath of a combined aqueous solution containing 10–20 % of an acidic catalyst and 3–18 % of an aldehyde with a provision that the acidic catalyst is contained in a greater amount than the aldehyde, raising the temperature of the bath gradually up to 50°–90° C. during a period of 0.5–10 hours, and then holding the bath at this temperature for 0–2 hours. The second stage of the curing treatment is carried out by immersing the fiber obtained from the first stage curing treatment in a curing bath of a com-

bined aqueous solution containing 0.3–7 % of an acidic or basic catalyst and 20–40 % of an aldehyde, i.e., that in which the content of aldehyde is greater, when the fiber is treated for 0.5–5 hours at a temperature of 70°–100° C. From the standpoint of the stability of pH and ease of operation, an acidic catalyst rather than a basic catalyst is preferred as the catalyst for this second curing bath. However, in the case where a greater number of crimps is desired as a result of the subsequent swelling treatment, preferred is a basic catalyst.

Since the content of catalyst is great in the aforesaid first stage curing bath and the degree to which the filament is swelled is low, the cure of the sheath layer proceeds while the crimps are inhibited. On the other hand, since the content of catalyst in the second stage curing treatment is small, a curing bath having a somewhat higher swellability is used, and the cure proceeds to the inner layer of the filament. Thus, a cured composite fiber having a degree of crosslinking of 5–45 mol %, and preferably 10–35 mol %, as hereinbefore specified, but in which the crimps are inhibited and present in a latent state is obtained.

Next, when this cured composite fiber is treated with a swelling agent, the desired uniform crimps are developed. The swelling treatment is suitably carried out by a procedure consisting of immersing the fiber in a swelling bath of a liquid ratio (fiber weight : swelling liquid weight) of 1 : 30–1 : 300 and holding it therein for 0.5–60 minutes at a temperature of 50°–120° C. Preferred swelling agents include alcohols of 1–4 carbon atoms such, for example, as methanol, ethanol and propanol, the ketones such as acetone and methyl ethyl ketone, and dioxane, dimethylformamide, dimethylacetamide, dimethyl sulfoxide, and the other polar solvents. For adjusting the degree of swelling so that it does not become too great, water can be added in an amount up to about 40 % by weight.

This swelling treatment is usually carried out by either the batch or continuous method immediately following the curing treatment. Further, when it is intended to make knit or woven fabrics having especially large number of crimps and abounding in elasticity by using this fiber, it is also possible to obtain such a fabric by a procedure consisting, say, of first developing in the fiber, after its cure, such number of crimps as will be suitable to permit the smooth operation of the spinning and knitting or weaving steps, and then, after the fibers have been knit or woven into a fabric, again submitting the fibers to a strong swelling treatment thereby obtaining a knit or woven product excelling in elasticity.

The self-crimping phenolic composite fiber of this invention, when treated under suitable tension with either wet or dry heat, can have part of its crimps removed, which crimps are made latent. These crimps which have been made latent can again be made manifest by submission to a suitable heat treatment under relaxed conditions.

The invention composite fiber, as a yarn spun from its staple form or as a continuous filament yarn, can be processed into heat resistant and flameproof textile products having the form of an elastic knit or woven product or a nonwoven fabric.

The following examples are given for more specifically illustrating the present invention. The parts and percentages in the examples are on a weight basis.

## EXAMPLE 1

1410 parts of phenol, 1180 parts of formalin (37 % aqueous solution), 20 parts of oxalic acid and 200 parts of methanol were reacted for 3 hours by heating at 100° C. with stirring, after which the reaction was terminated by the addition of a large quantity of cold water. The resulting phenolic resin was dissolved in methanol, and the unreacted phenol, formaldehyde and methanol and some water were distilled off by heating under reduced pressure to obtain a heat-meltable novolak resin of a number average molecular weight of 820. 950 parts of the so obtained novolak resin and 50 parts of nylon 12 (relative viscosity as measured in 0.5 % metacresol = 1.80) were mixed with stirring under a stream of nitrogen in an agitator-equipped autoclave for 3 hours at 210° C. under molten conditions. Then after debubbling the mixture under reduced pressure, the mixture was withdrawn from the bottom of the autoclave, and chips 0.25 mm in diameter and 0.3 mm long were prepared by the hot cut procedure. This is designated modified phenolic resin component A.

On the other hand, chips 0.25 mm in diameter and

5 60° C. in an 8 : 2 (volume) aqueous solution of methanol. After withdrawing the several fibers and washing them in water, they were dried at 80° C. under reduced pressure. The degree of crosslinking of the composite fiber was 32 mol %, and it had 8 crimps per inch.

10 Tests were continued for measuring the yarn quality and nonflammability of the several fibers. 0.1 gram of each of the fibers was taken and, after the filaments were laid together into a length of 19 centimeters, they were twisted 20 times and then folded in two at the middle. These samples were hung perpendicularly and exposed to a flame of an alcohol lamp by insertion of the sample one centimeter into the flame from the tip thereof. Twenty seconds later, the flame was removed, and the distance of carbonization was measured. Separately, 0.05 gram of each of the fibers was taken, and the filaments were likewise laid together into a length of 19 centimeters, twisted 20 times, and folded in two at the middle. The samples were exposed to the flame of an alcohol lamp for 5 seconds, then the flame was removed, and the fire continuance time of the fibers was determined. The results obtained are shown in Table 1.

Table 1

|                        | Fiber              | Spin-<br>nability | Crimp | Nonflammability                        |                                        | Yarn quality      |                        |
|------------------------|--------------------|-------------------|-------|----------------------------------------|----------------------------------------|-------------------|------------------------|
|                        |                    |                   |       | Carboni-<br>zation<br>distance<br>(cm) | Fire<br>continu-<br>ance time<br>(sec) | Tenacity<br>(g/d) | Elong-<br>ation<br>(%) |
| Invention<br>product   | Composite<br>fiber | good              | Yes   | 1.5                                    | 1.5                                    | 1.4               | 45                     |
| Control<br>product (B) | Single fiber       | poor              | no    | 1.5                                    | 1.0                                    | 1.3               | 32                     |
| Control<br>product (A) | Single fiber       | good              | no    | 2.5                                    | 4.5                                    | 1.3               | 41                     |

0.3 mm long were also prepared by the hot cut procedure from the aforesaid heat-meltable novolak resin. This is designated phenolic resin component B. Next, these two components of chip form were separately 40 melted in screw extruders at 200° C., following which they were compositely spun. The molten polymers were delivered by means of their respective gear pumps at a liquid feed ratio of 1/1 to a conventional composite spinneret and united in a side-by-side form and extruded through orifices 0.25 mm in diameter located at the face of the spinneret at 190° C. to form composite filaments, which were cooled in air and wound up at a spinning speed of 1000 meters per minute. The spinning was carried out satisfactorily with no breakage of yarn. By way of comparison, when the foregoing components, A and B were spun alone by feeding them separately to extruding spinning machines held at 200° C., it was possible to spin the component A satisfactorily, but in the case of component B, 55 yarn breakage occurred every few minutes.

Next, these several heat-meltable fibers were immersed in a combined aqueous solution bath of 18 % hydrochloric acid and 15 % formaldehyde at a bath ratio (fiber weight : bath liquid weight) of 1 : 100, after which the bath temperature was raised up to 95° C. during a period of 2 hours. At this time, helical crimps were only developed in the composite fiber. The reaction was continued for a further 6 hours at 95° C. to further the cure as well as to stabilize the crimps.

The several fibers were then withdrawn from the bath and repeatedly washed in cold water. This was followed by treating the fibers by immersion for 30 minutes at

45 50 It can be seen that the invention product is superior to the single fiber (B) in its spinnability and, on the other hand, excels in its nonflammability as compared with the single fiber (A).

## EXAMPLE 2

The heat-meltable composite fiber prepared in Example 1 was immersed at room temperature in a combined aqueous solution of 18 % hydrochloric acid and 2 % formaldehyde at a bath ratio of 1 : 100, after which the bath temperature was gradually raised up to 65° C. during a period of 5 hours, at which temperature the fiber was treated for a further 3 hours. Next, after withdrawing the fiber from the bath and washing it in water, it was dried under reduced pressure for 3 hours at 70° C. This fiber was then immersed at room temperature in a combined solution consisting of 1300 parts of hydrochloric acid (35.5 % concentrated hydrochloric acid), 1400 parts of formaldehyde (37 % aqueous solution), 240 parts of urea and 2840 parts of methanol at a bath ratio of 1 : 80, following which the bath temperature was raised up to 50° C. during a period of 2 hours, at which temperature the fiber was treated for a further 10 hours to prepare a composite fiber containing the urea bond and having a degree of crosslinking of 21 mol %. The tenacity of this fiber was 1.7 g/d and its elongation was 58 %. Further, it possessed gently sloping crimps at the rate of 21 crimps per inch. When this fiber was cut into 4-inch lengths and spun in customary manner, the spinnability was extremely satisfactory. Further, the so obtained spun yarn had an elongation of 8-12 %. Again, this fiber excelled in its heat resistance,

since its heat evolution starting point as determined by differential thermal analysis was 330° C., a high value. Thus, there is an improvement of about 110° C. as compared with a fiber not containing the urea bonds.

### EXAMPLE 3

Chips of the heat-meltable novolak resin obtained in Example 1 and designated therein as component A and nylon-66 chips ( $[\eta] = 1.02$  as measured in metacresol at 30° C.) in a prescribed ratio to the former were introduced into a rotary dryer and mixed in their chip state to prepare the component C.

Next, a composite fiber was spun from the components C and B by operating as in Example 1. The resulting fiber was then immersed at room temperature in a combined solution of 15% hydrochloric acid and 16% formaldehyde, after which the temperature of the bath was raised up to 90° C. during a period of 2 hours, at which temperature the fiber was treated for 5 minutes. After withdrawing the fiber from the bath and water-washing, it was immersed at 40° C. in a combined aqueous solution containing 30% of formaldehyde and 2.8% of ammonia, after which the temperature of the bath was raised up to 95° C. during a period of 1 hour, at which temperature the fiber was cured for one hour. The fiber was then withdrawn from the bath, water-washed and dried, after which it was measured for its nonflammability by the same method as described in Example 1. Further, the elongation and recovery of the fiber were determined as follows:

$$\text{Elongation (\%)} = \frac{L_1 - L_0}{L_0} \times 100$$

$$\text{Recovery (\%)} = \frac{L_1 - L_2}{L_1 - L_0} \times 100$$

where

$L_0$  = original length (cm),

$L_1$  = length one minute after loading with a 0.15 g/d load (cm) and

$L_2$  = length one minute after removal of load (cm).

The results obtained are shown in Table 2.

Table 2

| Content of<br>nylon 66 in<br>component C | Spinnability | Nonflammability                        |                                        | Elongation and<br>recovery |                 |
|------------------------------------------|--------------|----------------------------------------|----------------------------------------|----------------------------|-----------------|
|                                          |              | Carboni-<br>zation<br>distance<br>(cm) | Fire con-<br>tinuance<br>time<br>(sec) | Elongation<br>(%)          | Recovery<br>(%) |
| Control<br>product                       | 0.3          | poor                                   | 1.5                                    | 1.0                        | 15              |
| Invention<br>product                     | 0.5          | fair                                   | 1.5                                    | 1.0                        | 35              |
| "                                        | 1            | "                                      | 1.5                                    | 1.5-2.0                    | 55              |
| "                                        | 2            | good                                   | 1.7                                    | 1.5-2.0                    | 78              |
| "                                        | 5            | "                                      | 1.7                                    | 1.5-2.0                    | 110             |
| "                                        | 7            | "                                      | 1.8                                    | 2.0                        | 120             |
| "                                        | 10           | "                                      | 2.0                                    | 2.5                        | 140             |
| "                                        | 30           | "                                      | 2.9                                    | 3.0                        | 150             |
| Control<br>product                       | 40           | "                                      | 4.2                                    | 5.5                        | 97              |

It is apparent from Table 2 that at least 0.5% of nylon-66 is required when considered from the standpoint of the spinnability and the elongation and recovery rates. On the other hand, it is seen that from the standpoint of nonflammability an amount in excess of 30% was not desirable. Further, it is seen that the amount of nylon-66 was preferably 1-10%, and most preferably 2-7%.

On the other hand, in the case where 10% of nylon was added, as indicated above, but the composite fiber obtained was one in which the phenolic resin nylon-66 was used as the core with an eccentrically disposed sheath disposed enveloping the core, which fiber was then cured in exactly the same manner to obtain a phenolic composite fiber, the elongation was 65% and elongation recovery was 92%. While the crimp properties were thus somewhat inferior to the side-by-side form, good results were obtained with respect to the fiber's nonflammability in that the carbonization distance was 1.5 cm and the fire continuance time was 1.5-2.0 seconds.

### EXAMPLE 4

Coal-tar pitch and the component B prepared in Example 1 were mixed at a ratio of 30/70 (weight %) to obtain a modified novolak (component D). The so obtained component D and the component B itself were then spun into a side-by-side type composite fiber at a ratio of union of D/B = 7/3 by operating as in Example 1 and thereafter cured by operating as in said example to obtain a self-crimping phenolic composite fiber.

The so obtained composite fiber was highly nonflammable as is apparent from the results obtained when it was tested as in Example 2, the carbonization distance being 1.5 cm and the fire continuance time being 0-0.5 second.

### EXAMPLE 5

1410 parts of phenol, 1180 parts of formalin (37% aqueous solution), 20 parts of oxalic acid and 50 parts of methanol were reacted for 3 hours by heating at 95° C. with stirring, following which the reaction was terminated by the addition of a large quantity of water. The resulting resin was then treated at 150° C. under reduced pressure to distill off the water and unreacted monomers to obtain a heat-meltable novolak resin of a number average molecular weight of 860. When this resin was passed through a stainless steel mesh of 10-micron size under molten conditions, the resin was formed into beadlike particles. This is designated com-

ponent B<sub>1</sub>.

Next, 95 parts of this beadlike phenolic resin and 5 parts of chips of nylon 12 (relative viscosity as measured in 0.5% methanol of 1.65) were mixed thoroughly in a rotary dryer to obtain a mixture (designated component A<sub>1</sub>), which was fed to a melt-extruding composite spinning machine of 20-mm diameter held

at 200° C. where it was spun into a composite fiber. That is, the foregoing mixture (component A<sub>1</sub>) and the phenolic resin (component B<sub>1</sub>) were fed to a usual composite spinneret at a liquid feed ratio of 1/1 by means of gear pumps and, after being united into a side-by-side form, were extruded from orifices of 0.5-mm diameter disposed at the 180° C. spinneret face, followed by cooling in air and winding up at a spinning speed of 800 meters per minute. The spinning was carried out satisfactorily with no yarn breakage. By way of comparison, the foregoing components A<sub>1</sub> and B<sub>1</sub> were separately fed to an extruding spinning machine held at 200° C. and separately spun. While the spinning in the case of the component A<sub>1</sub> could be carried out satisfactorily, yarn breakage occurred every few minutes in the case of the component B<sub>1</sub>.

Next, the heat-meltable composite fiber obtained by compositely spinning the aforesaid components A<sub>1</sub> and B<sub>1</sub> was separated from the bobbin and immersed at room temperature in a combined aqueous solution consisting of 17 % hydrochloric acid and 12 % formaldehyde at a bath ratio of 1 : 40, following which the temperature of the bath was raised up to 70° C. during a period of 2.5 hours, at which temperature the reaction was continued for a further 30 minutes. The sheath layer of the fiber was cured by this treatment, but there was no manifestation of crimps.

The so obtained partially cured fiber was immersed at 700° C. in a combined aqueous solution consisting of 3 % hydrochloric acid and 35 % formaldehyde, after which the temperature of the bath was raised up to 95° C. during a period of 30 minutes followed by continuing the reaction for a further 2 hours to further the cure of the fiber to the inner layer thereof. The degree of crosslinking was 32 mol %. Further, there was some development of gentle waves in the resulting cured fiber (on the order of about one wave per 4 inches). This cured fiber was then introduced into methanol at a liquid ratio of 1 : 200 and treated for 10 minutes at

5  
10  
15  
20  
25  
30  
35  
40  
45  
50  
55  
60  
65  
66  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880  
8885  
8890  
8895  
8900  
8905  
8910  
8915  
8920  
8925  
8930  
8935  
8940  
8945  
8950  
8955  
8960  
8965  
8970  
8975  
8980  
8985  
8990  
8995  
9000  
9005  
9010  
9015  
9020  
9025  
9030  
9035

properties, said method comprising melt-spinning (A) a modified phenolic resin obtained by melt blending a heat-meltable uncured novolak resin with 0.5-30 % by weight, based on the total weight of the mixture, of a heat-meltable fiber-forming resin selected from polyamide resin, polyester resin, polyurethane resin or polyolefin resin, and (B) a heat-meltable uncured novolak resin, said melt-spinning being carried out such that the components (A) and (B) are united in an eccentric or side-by-side relationship, and thereafter curing the phenolic resin component contained in the resulting heat-meltable composite fiber.

2. A method of producing a self-crimping phenolic composite fiber having heat-resistant flameproof properties, said method comprising melt-spinning (A) a modified phenolic resin obtained by melt blending a heat-meltable uncured novolak resin with 0.5-30 % by weight, based on the total weight of the mixture, of a heat-meltable fiber-forming resin selected from polyamide resin, polyester resin, polyurethane resin or polyolefin resin, and (B) a heat-meltable uncured novolak resin, said melt-spinning being carried out such that the components (A) and (B) are united in an eccentric or side-by-side relationship, curing the phenolic resin component contained in the resulting heat-meltable composite fiber and thereafter treating said fiber with a swelling agent.

3. The method of claim 2 wherein said heat-meltable fiber-forming resin is contained in said modified phenolic resin (A) in an amount of 1-10 % by weight.

4. The method of claim 2 wherein said heat-meltable fiber-forming resin is contained in said modified phenolic resin (A) in an amount of 2-7 % by weight.

5. The method of claim 2 wherein the weight ratio of said modified phenolic resin (A) to said heat-meltable uncured novolak resin (B) ranges between 10:90 and 90:10.

6. The method of claim 2 which comprises carrying out the cure of the phenolic resin component contained in the heat-meltable composite fiber until a degree of crosslinking of 5-45 mol % is achieved.

7. The method of claim 2 which comprises carrying out the cure of the phenolic resin component contained in the heat-meltable composite fiber until a degree of crosslinking of 10-35 mol % is achieved.

45

8. The method of claim 2 wherein said heat-meltable fiber-forming resin is a polyamide.

9. The method of claim 2 wherein said curing treatment is carried out by a two-stage process consisting of a precuring and a curing step.

10. The method of claim 9 which comprises carrying out the curing treatment by a two-stage process consisting of a precuring and a curing step, said precuring step being carried out using a curing bath in which the content of the acidic catalyst is greater than that of the aldehyde, and said curing step being carried out using a curing bath in which the content of the acidic or basic catalyst is less than that of the aldehyde.

11. The method of claim 1 wherein said heat-meltable fiber-forming resin is contained in said modified phenolic resin (A) in an amount of 1-10 % by weight.

12. The method of claim 1 wherein said heat-meltable fiber-forming resin is contained in said modified phenolic resin (A) in an amount of 2-7 % by weight.

13. The method of claim 1 wherein the weight ratio of said modified phenolic resin (A) to said heat-meltable uncured novolak resin (B) ranges between 10:90 and 90:10.

14. The method of claim 1 which comprises carrying out the cure of the phenolic resin component contained in the heat-meltable composite fiber until a degree of crosslinking of 5-45 mol % is achieved.

15. The method of claim 1 which comprises carrying out the cure of the phenolic resin component contained in the heat-meltable composite fiber until a degree of crosslinking of 10-35 mol % is achieved.

16. The method of claim 1 wherein said heat-meltable fiber-forming resin is a polyamide.

17. The method of claim 1 wherein said curing treatment is carried out by a two-stage process consisting of a precuring and a curing step.

18. The method of claim 17 which comprises carrying out the curing treatment by a two-stage process consisting of a pre-curing and curing step, said precuring step being carried out using a curing bath in which the content of the acidic catalyst is greater than that of the aldehyde, and said curing step being carried out using a curing bath in which the content of the acidic or basic catalyst is less than that of the aldehyde.

\* \* \* \* \*

50

55

60

65